

## UNITED STATES PATENT OFFICE

WALTER H. RANDALL, OF WATERVILLE, MAINE, ASSIGNEE, BY MESNE ASSIGNMENTS,  
TO FIDELITY TRUST COMPANY, OF PORTLAND, MAINE, A CORPORATION OF MAINE,  
TRUSTEE

## ART OF SIZING

No Drawing.

Application filed June 24, 1929. Serial No. 373,477.

In the sizing of pulp stocks, particularly for waterproof or greaseproof results, there has been much general difficulty in introducing the size to get uniform distribution. This has been conspicuously apparent where such stocks have been used in die forming operations as by suction or pressure deposit on perforate or foraminous moulding dies.

The general problem has been to introduce 10 the rosin, wax, paraffin, or other sizing into the pulp in such dispersed state that it would not coagulate or otherwise gather in particles on the die and thus clog its perforations and retard or block its efficiency.

15 Previous methods have involved the saponification or emulsification of the size, but in accordance with my concept, I mechanically disperse the size. For example, rosin, wax, paraffin or similar sizing ingredients either 20 singly or in combination, have not been dispersed without complicated chemical treatment. I propose by my present method to mix this mechanically in a fibrous mixture 25 medium whereby to provide a complete mixture without including any extraneous or reactive concomitants.

To this end my present invention contemplates a method of effecting such a mixture and to illustrate this I will discuss a methodical procedure by which such sizing may be 30 accomplished.

To distribute a sizing such as rosin, wax, or other sizing ingredients, in a pulp solution as ground wood pulp or ground wood and 35 chemical fibre pulp, or other fibrous pulp materials, or any of them in combination, I effect first a mechanical mixture as heretofore suggested. The mechanical mixture of such a substance, as rosin, wax, paraffin or 40 the like, in fibre presents some difficulties of peculiar nature.

I find that such mixtures can be most readily effected where the fibrous mixture medium is a dry bat or sheet, preferably somewhat compacted. Such fibrous mixture medium may be wood fibre, a vegetable fibre, a chemical fibre as distinguished from an untreated wood fibre, or I may use any other fibre possessing the equivalent qualities.

45 50 The size and fibre may be worked together

by rolling or rubbing or similar operations, but in so doing the fibre should be in a dry state to which the sizing ingredient should preferably be added in a melted condition. The mixing is carried on until the sizing ingredient has been completely mixed on the fibre surface and preferably in amount of approximately 25% of the sizing ingredient to fibre. Where a bat or sheet is developed as a basis of mixture, the size will be absorbed by a progressive submersion by which any air in the bat is forced out. There is preferably in the ultimate product a phase of water dispersion so that by continued or supplemental treatment with water, the resultant size is in sludge or fluid pulp form. The sizing is made from a bat or sheet. It is usually convenient to reduce it to a fluid consistency so that it can be more conveniently added to the pulp stock solution. In doing this it can simply be beaten up with water or with some of the pulp stock solution to which it is to be added.

All such stocks are preferably reduced 55 to a fluid state and as best adapted to their production I provide a working basis at about 10% density as best for water dispersion.

In order to produce the highest perfection in my mechanically mixed size, I preferably carry its treatment to such a point that the sizing material is incorporated into the fibre itself as distinguished from being merely on the surface. There seem to be three conditions of the fibre worked according to my process. These may or may not represent states or stages, although with some fibres and some sizings, the fibre doubtless passes through these successive conditions in successive stages of the process. The first condition to be noted is where the size is wholly on the surface of the fibre. This may be due to the hardness of the sizing or to the impermeability of the fibre used or to a minimum degree of working the sizing and fibre together. The second condition seems to be where the fibre has taken the sizing into its surface area to a slight depth without complete penetration. The third condition is apparently where the sizing has 60 65 70 75 80 85 90 95 100

completely penetrated the fibre so as to amount to an impregnation. This possibly may represent a filling of the fibre cells or interstices. This may depend on the kind of fibre used and the kind of sizing used and also to the degree of working or manipulation of the materials. This complete impregnation represents the most successful type of dispersion as it is absolutely free from any tendency to flocculate or bunch in the mixture. The type first described while successful under ordinary conditions may have a slight tendency to gather in bunches or mass.

Such a sizing ingredient comprising free vegetable fibre mechanically mixed preferably with untreated size is capable of an intimate and complete mixture with ordinary ground wood pulp or other pulp solutions to produce a stock from which articles of most advantageous characteristics may be fabricated.

For example, such a sized stock can be run on a suction die machine in moulding articles such as plates or other containers in which water-proofness or grease-proofness is desired. Unlike other sized stocks there is no clogging of the die perforations or screen interstices and the resultant articles, after drying at size fusing temperatures, are more perfectly sized and structured than any with ordinary sizing. In drying, the fusion of the flux seems more complete and efficient than in any previously sized stock.

Without intending to limit myself, I offer the further consideration. Where chemically treated fibre is used as the fibrous mixing medium, there seems possible a hydration of the fibre which aids materially in the mixing of the size. This may be only a partial or surface hydration, but it seems to assist the attenuation of the size dispersion. The fibre should be preferably dry and as free from moisture as possible. This is apart from any so-called hydration.

It will also be understood that where I use the term untreated size that I intend thereby to differentiate from emulsified or saponified sizings such as have been heretofore used. The size may be slightly saponified if desired and as before stated the size used may in itself be a blend or composition. The point is that the size used is in a state of substantial mechanical mixture in or on the fibre surface and is in an extremely attenuated state and capable of being carried by its mixing fibre throughout the pulp solution to be sized to effect a complete distribution and without danger of coagulation or flocculation. These and other reasonable interpretations of terms are to be understood as within the following claims.

What I therefore claim and desire to secure by Letters Patent is:

1. That method of sizing an aqueous pulp

solution, consisting in mixing into such solution a mixture of dry fibres and an unemulsified size.

2. That method of sizing an aqueous pulp solution, consisting in mixing into such solution a mixture of partially hydrated dry fibres and an unemulsified size. 70

3. That method of preparing a sizing mixture, consisting in mechanically mixing dry fibres and an untreated size. 75

4. That method of sizing a pulp solution, consisting in first dry mixing fibres and an untreated sizing, and in thereafter mixing the sized fibres into an aqueous pulp solution. 80

5. That method of sizing an aqueous pulp solution, consisting in first distributing an untreated sizing on a dry fibre sheet, in thereafter disintegrating the sheet to effect a complete mixture of the fibre with the sizing thereon to maintain the sizing in an attenuated state, and in finally mixing the sized fibres into the aqueous pulp solution. 85

6. The method of sizing an aqueous pulp solution consisting in first mechanically distributing an untreated sizing on a surface hydrated dry fibre to effect an adherent attenuated mixture thereof, and in thereafter mixing the sized fibres into the aqueous pulp solution. 90

7. That step in the method of sizing an aqueous pulp solution, which consists in mixing into the pulp solution a dry mixture of unmodified size and hydrated fibres. 95

8. The method of sizing an aqueous pulp solution which consists in first dry mixing fibres and a sizing ingredient in unheated condition, and in thereafter mixing said mixture with unsized fibres in the presence of water to form an aqueous pulp solution, 100 consisting of an unheated mixture of sized and unsized fibres. 105

9. The method of forming a grease-proofed molded article, which consists in first dry mixing fibres and a sizing ingredient in unheated condition, in thereafter mixing said mixture with unsized fibres in the presence of water to form an aqueous pulp solution consisting of an unheated mixture of sized and unsized fibres, die molding from such unheated solution an article of the desired size, shape and consistency and in finally drying such molded article at a temperature sufficiently high to effect the transfer of the size from the sized fibres to the unsized fibres. 110 115 120

In testimony whereof I affix my signature.  
WALTER H. RANDALL.